

## UNITED STATES PATENT OFFICE

2,388,439

## CUTTING OIL

Leslie R. Raymond, Santa Ana, Calif., assignor to  
 A. S. Cowie & Co., Los Angeles, Calif., a corporation of California

No Drawing. Application August 21, 1944,  
 Serial No. 550,485

6 Claims. (Cl. 252—42.7)

This invention relates to cutting oils for use in metal cutting, drilling, reaming, or other machining operations.

Cutting oils are used to perform several important functions in such operations. They act to provide lubrication between the tool and the work and also to dissipate heat and thus prevent overheating of either the tool or the work. By reason of these effects they reduce the power consumed, increase the life of the tools, and provide smoother and more perfect surfaces on the work.

Many different types of compositions have been used for cutting oils. Mineral oils have been used for light duty cutting, where the requirements for lubrication and cooling are not severe, but have not been found satisfactory for more difficult machining operations. Where the requirements for cooling and lubrication are severe, the compositions used have generally consisted principally of animal or vegetable oils, and sulphur is often added for the purpose of increasing the film strength. Vegetable or animal oils have certain disadvantages, however, including objectionable odor and a tendency to become rancid.

The principal object of this invention is to provide a cutting oil which effectively performs the above mentioned functions and which does not require the use of animal or vegetable oil or the addition of sulphur.

A particular object is to provide a cutting oil composition which provides a highly effective lubricating and protective film on both the work and the tool.

The cutting oil of my present invention consists principally of mineral lubricating oil and naphthenic acid and contains, in addition, a relatively small proportion of metallic naphthenate dissolved or colloidally dispersed therein.

The term mineral lubricating oil is used herein to designate a petroleum oil, either paraffin base or naphthene base, which has some lubricating value, including products commonly used as lubricating oils as well as oils of lower boiling point and lower viscosity, such as gas oil, kerosene or kerosene distillate.

Naphthenic acids are derived from naphthene base petroleum oils and usually comprise a number of different compounds rather than a single compound. The naphthenic acids which I have found suitable for purposes of my invention have an acid number from about 75 to about 375, although the best results are usually obtained by the use of a naphthenic acid having an acid number between about 100 and 250. For exam-

ple, I have obtained excellent results with a naphthenic acid having an acid number of approximately 100, which would correspond approximately to an acid having the formula



This of course is not the true formula but represents approximately the average formula of the acids present in the material.

10 The proportions of mineral lubricating oil and naphthenic acid are subject to considerable variation. These materials are freely miscible with or soluble in one another in any proportions. In the cutting oil of my invention the proportions 15 may, for example, vary between about 5% and 75% by volume of naphthenic acid to between about 95% and 25% of mineral lubricating oil. For most purposes compositions containing from about 10% to about 50% by volume of naphthenic acid give excellent results.

20 The mineral lubricating oil and naphthenic acid are mixed together to form a solution and the metallic naphthenate may, if desired, be separately prepared and added to the resulting solution. According to a preferred procedure, however, I may form the metallic naphthenate in the lubricating oil-naphthenic acid solution by contact thereof with a compound of the desired metal which will react with a portion of the 25 30 naphthenic acid to form metallic naphthenate.

Various metallic naphthenates may be employed such as those of magnesium, calcium, aluminum, lead, manganese, copper, iron, cobalt or nickel. Mixtures of two or more of these metallic naphthenates may also be used.

35 The proportion of metallic naphthenate in the cutting oil composition should be at least  $\frac{1}{2}\%$  by weight, and I prefer to use from about 1% to about 5% metallic naphthenate.

40 Naphthenates of the above mentioned metals may be prepared by heating the oxide of such metal with naphthenic acid, or by reacting sodium naphthenate with a solution of a soluble salt of the metal. For example, in preparing 45 magnesium naphthenate I may heat magnesium oxide with naphthenic acid, or I may first react sodium hydroxide with naphthenic acid to form sodium naphthenate and then subject the latter to contact with a solution of magnesium sulphate or magnesium chloride to form magnesium naphthenate.

50 In the making of my cutting oil composition, the lubricating oil and naphthenic acid may be either crude or refined. Since there is considerable difference in price between the crude and

refined products, I generally prefer to use the cheaper, unrefined materials and to refine them by treatment with sulphuric acid to remove asphaltic or gum-forming impurities. In the refining process, the materials may be treated separately and subsequently mixed, or the mixture may be made prior to the refining process, a procedure which I prefer. As an example of this procedure, I first mix thoroughly in the desired proportions, a crude lubricating stock and a crude naphthenic acid of the desired acid number. This mixture is then treated with from one to ten pounds of 66° Bé. sulphuric acid per barrel (of 42 U. S. gallons) of the mixture, and the whole thoroughly agitated for ten to fifteen minutes, which is sufficient to remove the impurities but not sufficient to cause sulfonation of the naphthenic acids, since it is well known that these sulfonation reactions proceed quite slowly. After the agitation, the acid sludge is allowed to settle and is drawn off from the bottom of the container or the oil mixture may be decanted from the sludge.

The resulting refined mixture may then be subjected to filtration in any desired manner to remove any suspended acid sludge or any other undissolved impurities, and is preferably then treated with caustic soda solution to neutralize any free sulphuric acid or sulphur dioxide, after which the desired proportion of metallic naphthenate produced as described above may be added and the whole mixture thoroughly agitated to uniformly distribute the metallic naphthenate, either in solution or in the form of a colloidal dispersion. As an alternative, the metallic naphthenate may be incorporated in the mixture prior to the filtration step.

An example of a cutting oil prepared by mixing and treating the ingredients as described above is one containing 25 parts by volume of naphthenic acid to 75 parts of mineral lubricating oil together with 2 to 2½% by weight of metallic naphthenate based on the total weight of the mixture. The metallic naphthenate may, for example, be magnesium naphthenate, calcium naphthenate, or aluminum naphthenate.

According to the preferred procedure mentioned above, metallic naphthenate may be formed in the refined lubricating oil-naphthenic acid mixture by contact of such mixture with an oxide, silicate, or other reactive compound of the desired metal. In following this procedure, I find it especially advantageous to employ a compound of the desired metal which is also capable of acting as a filter aid and also as an adsorbent material for decolorizing the mixture.

As a specific example of this preferred method of preparation, a mixture is made containing 20% by volume of naphthenic acid and 80% by volume of mineral lubricating oil. This mixture is treated with 66° Bé. sulphuric acid and thoroughly agitated to remove asphaltic and gum-forming constituents, after which the sludge is allowed to settle and is drawn off. The refined mixture is then heated to approximately 130° F., and a hydrated magnesium silicate is added in the proportion of about 3% by weight of the mixture. The mixture is then agitated well for a sufficient period to cause partial reaction between the magnesium silicate and the naphthenic acid to form the desired proportion of magnesium

naphthenate, for example, for about two to four hours. The mixture is then filtered to remove the unreacted magnesium silicate and other undissolved solids.

5 The magnesium silicate is preferably one which has a high adsorbent power, such as a synthetic hydrated magnesium silicate sold under the trade name of Magnesol, which acts not only to produce magnesium naphthenate in the solution by partial reaction with the naphthenic acid but also as a filter aid and adsorbent to remove both suspended solids and color from the mixture.

A cutting oil composition prepared by the specific procedure described above, using Magnesol, 15 was found to contain about 1½% of magnesium naphthenate together with somewhat less than 1% of iron naphthenate, the latter probably resulting from reaction of the naphthenic acid with the iron vessels and equipment employed in the 20 process.

It will be understood of course that other materials in addition to those mentioned above may also be added to the composition if desired, without departing from the scope of my invention. 25 However, I have found that compositions containing only the above mentioned ingredients within the specified ranges give very excellent results when used as cutting oils. The manner of applying and using such compositions may be 30 essentially the same heretofore employed with other cutting oil compositions.

I claim:

1. A cutting oil consisting principally of mineral lubricating oil and naphthenic acid in proportions between 5% and 75% naphthenic acid to between 95% and 25% mineral lubricating oil, by volume, and also containing from ½% to about 5% by weight of metallic naphthenate.

2. A cutting oil consisting principally of mineral lubricating oil and naphthenic acid in proportions between 5% and 75% naphthenic acid to between 95% and 25% mineral lubricating oil, by volume, and also containing from 1% to 5% by weight of metallic naphthenate.

3. A cutting oil consisting principally of mineral lubricating oil and naphthenic acid in proportions between 10% and 50% naphthenic acid to between 90% and 50% mineral lubricating oil, by volume, and also containing from ½% to about 5% by weight of metallic naphthenate, said naphthenic acid having an acid number between about 75 and 375.

4. A cutting oil consisting principally of mineral lubricating oil and naphthenic acid in proportions between 10% and 50% naphthenic acid to between 90% and 50% mineral lubricating oil, by volume, and also containing from 1% to 5% by weight of metallic naphthenate.

5. A cutting oil consisting principally of mineral lubricating oil and naphthenic acid in proportions between 5% and 75% naphthenic acid to between 95% and 25% mineral lubricating oil, by volume, and also containing from ½% to about 5% by weight of magnesium naphthenate.

6. A cutting oil consisting principally of mineral lubricating oil and naphthenic acid in proportions between 5% and 75% naphthenic acid to between 95% and 25% mineral lubricating oil, by volume, and also containing from ½% to about 5% by weight of calcium naphthenate.

LESLIE R. RAYMOND.